

E. SCHAAF & S. G. MARTIN.  
METHOD OF RECOVERING COPPER FROM ITS ORES.  
APPLICATION FILED AUG. 27, 1909.

1,069,981.

Patented Aug. 12, 1913.



attest:  
A. G. Fletcher.  
E. L. Wallace -

Trenton,  
Edward School.  
Stephen G. Martin.  
By Higdon & Longan.  
atty 3.

# UNITED STATES PATENT OFFICE.

EDWARD SCHAAF, OF ST. MARYS, MISSOURI, AND STEPHEN G. MARTIN, OF CHICAGO, ILLINOIS, ASSIGNEES OF ONE-THIRD TO WILLIAM O. BARTHOLOMEW, OF ST. LOUIS, MISSOURI.

## METHOD OF RECOVERING COPPER FROM ITS ORES.

1,069,981.

Specification of Letters Patent.

Patented Aug. 12, 1913.

Application filed August 27, 1909. Serial No. 514,847.

To all whom it may concern:

Be it known that we, EDWARD SCHAAF and STEPHEN G. MARTIN, both citizens of the United States, and residents of St. Marys, 5 Missouri, and Chicago, Illinois, respectively, have invented certain new and useful Improvements in Methods of Recovering Copper from Its Ores, of which the following is a specification containing a full, clear, and 10 exact description, reference being had to the accompanying drawings, forming a part hereof.

Our invention relates to a new and useful method of recovering copper from its 15 ores, the object of our invention being to obtain copper wholly or in part in its metallic state from its ores by a process of leaching, solution, heat, pressure, vaporizing and precipitation by a condensation.

20 We employ, in carrying out our process, the use of a gaseous medium containing peroxid and lower oxids of nitrogen  $N_2O_4$ ,  $N_2O_3$ ,  $N_2O_2$  and  $N_2O$ , that is a gas formed by passing ordinary atmospheric air through 25 a flaming electric arc or through an electric flaming discharge.

When ordinary atmospheric air is passed through an electric flaming discharge a gaseous medium is formed which consists 30 largely of pure air and peroxid and lower oxids of nitrogen, and, we have found out, by experiment, that such a gaseous medium exercises a sort of selective function toward the copper content of any copper solution 35 amenable to our treatment.

By our improved method, we are enabled to recover practically all of the copper contained in any ore that is capable of being forced into solution, and whether the solution be neutral or acid by our process precipitation of the copper is effected apparently instantaneously and the solvent is at once freed of its metal burden by the following reaction:  $2CuSO_4 + (N_2O_3$ , 45 and air)  $+ 3H_2O + \text{heat and pressure} = 2Cu + 2H_2SO_4 + 2HNO_3$ . When the solvent solution is acid it may be re-used.

The operation of our process of metal recovering is a continuous one so long as the 50 supply of the cupric or cuprous solution is uninterruptedly fed to the vaporizer.

In order to describe more clearly our improved method, reference is had to the accompanying drawing, wherein:

1 indicates the supply tank adapted to contain the cupric or cuprous solution.

2 indicates a tank into which the copper solution, from the tank 1, is passed through a pipe 3 in which is located a valve 4 for controlling the passage of the cuprous solution from tank 1 to tank 2. Located in the tank 2 is a steam coil 5, one end of which may be attached to any suitable source of steam supply and the opposite end 6 is the exhaust end of the coil. The steam coil 5 is for heating the cuprous solution.

As heretofore stated, we employ as agent in our process a gaseous medium containing peroxid and the lower oxids of nitrogen. This gaseous medium is produced by means 70 of a pair of electrodes 7 and 8 mounted in a housing 9 and form the terminals of an electric circuit which may be passed through the conducting wires 10 and 11.

In practice it is found preferable to employ a current having high amperage and a relative low voltage and any form of generator capable of producing such a current may be used. Atmospheric air is forced through the housing 9 and through the flaming electric discharge between the electrodes 7 and 8 by means of a fan 12, and the gaseous medium, thus formed, which consists of pure air and peroxid and the lower oxids of nitrogen, passes through the pipe 13 and into the tank 2. Secured to the bottom 85 of the tank 2 is a pipe 14 in which is located a valve 15 and the lower end of the pipe 14 terminates in a perforated head 16 which causes the fluid passing through it to be diffused in a series of small screens or jets.

17 indicates a vaporizing tank in which the perforated head 16 is located. This tank is of sufficient strength to stand a high degree of pressure and is suitably lined so as not to be affected by the solution. Secured to one side of the tank 17 is a pipe 18 in which is located a valve 19, said pipe 18 being adapted to be secured to any suitable source of steam supply under pressure. Secured to the tank 17 is a pipe 20, one end of which terminates in a condensing chamber 21, said condensing chamber being provided with valves 22 and 23.

24 and 25 indicate similar condensing 105 chambers provided with man-holes 26. Leading from the condensing chamber 21 into the condensing chamber 24 is a pipe 27

and leading from the condensing chamber 24 into the condensing chamber 25 is a pipe 28. Each one of the condensing chambers 24 and 25 being provided with cut-off valves 29, 30, 31 and 32 respectively.

33 indicates water-level pipes or tubes which are connected to the chambers 21, 24 and 25, the chamber 21 also being provided with a safety valve 34.

10 The operation of our process is as follows: The ore from which the copper is to be removed is first crushed or ground in any of the well known methods and is then leached or otherwise digested with a suitable solvent 15 of sufficient strength to dissolve all of the copper present in the ore that is capable of being forced into solution. The solution of copper is then placed in the tank 1 and this solution is then conveyed or passed to tank 2 and is therein heated to any suitable 20 degree of temperature. While the solution of copper is being heated it, the said solution, is treated with a gaseous medium containing peroxid and lower oxids of nitrogen 25 through the pipe 13. In other words said solution is charged with said gaseous medium. The charged solution is then passed into the pressure tank 17 and if the same does not flow rapidly enough into said tank 30 we may employ a pump 35 to increase the flow. The charged solution passes through the perforated head 16 in the form of small jets or sprays, and as it is emitted from said head steam is admitted into said tank 17 35 through the pipe 18 under pressure, when decomposition into metallic copper of the copper salt of said charged solution occurs and the products of said decomposition, together with the vaporized water of the solution, are forced over through pipes 20, 27 40 and 28 into the condensing chambers 21, 24 and 25, where precipitation of the metal in a finely divided or comminuted state takes place, the greater portion of the precipitate 45 taking place in the chamber 21; each chamber 21 and 24 being provided with baffle plates 36 and 37 which have a tendency to check or resist the passage of light particles of material beyond the first condensing 50 chamber 21.

The precipitated metal is collected in the chambers lying below the uppermost valves in each condensing chamber until they have been practically filled and then they are discharged into a car 38 or other receptacle by means of the lowermost of the slide valves carried by the condensing chambers, and the steam admitted to the pressure tank 17 being finally exhausted through the pipe 39.

60 While we have shown one form of apparatus by means of which our process may be carried out, various apparatus may be designed for carrying out our process.

The essential features of our process are 65 in the employment of a gaseous medium

containing peroxid and the lower oxids of nitrogen combined with heat, pressure and the precipitation of the metal by condensation. In other words, the essential features of our invention are the treatment of a solution of copper with heat and pressure and a gaseous medium containing peroxid and lower oxids of nitrogen and the condensation of the vapor.

70 While we have shown an electrical apparatus for producing the gaseous peroxid and lower oxids of nitrogen, we may produce this gas chemically, and while we have shown a liquid in the condensing chambers for effecting the condensation, we may use any suitable liquid as a precipitant with or 75 without re-agent.

80 The pump 35 may be used for forcing the solution from the tank 2 into the vaporizing chamber 17, the back pressure being controlled by means of a check valve 40, the 85 passage of the solution to the pump being controlled by means of a valve 41.

We claim:

1. The herein described process of recovering copper from its ores, which consists first in converting the copper content of the ore to a solution, charging said solution with a gaseous medium containing peroxid of nitrogen and the lower oxids of 90 nitrogen, and subjecting said charged solution to the action of a hot fluid blast agent.

100 2. The herein described process of recovering copper from its ores, which consists in converting the copper content of the ore to a solution, treating said solution with a gaseous medium containing peroxid of nitrogen and the lower oxids of nitrogen, and subjecting said solution thus treated to 105 the action of a hot fluid blast agent.

110 3. The herein described process of recovering copper from its ores, which consists in converting the copper content of the ore to a solution, heating said solution, charging said heated solution with peroxid of nitrogen and the lower oxids of nitrogen gas and subjecting said solution thus charged to the action of steam.

115 4. The herein described process of recovering copper from its ores, which consists in converting the copper content of the ore to a solution, charging the copper solution with gaseous peroxid of nitrogen and the lower oxids of nitrogen; and subjecting 120 said solution to heat and pressure.

125 5. The herein described process of recovering copper from its ores, which consists in converting the copper content of the ore to a solution, treating the copper solution with gaseous peroxid of nitrogen and the lower oxids of nitrogen; and subjecting said solution to the action of a fluid heating medium under pressure.

130 6. The herein described process of recov-

ering copper from its ores, which consists in converting the copper content of the ore to a solution, charging said solution with peroxid of nitrogen and the lower oxids of 5 nitrogen; and then applying heat to said solution.

7. The herein described process of recovering copper from its ores, which consists in converting the copper content of the ore 10 to a solution, charging said solution with peroxid of nitrogen and the lower oxids of nitrogen; and applying heat and pressure to said charged solution.

8. The process of recovering copper from 15 its ores by the wet method, which consists in leaching the ore with a suitable solvent, treating the resulting solution with peroxid of nitrogen and the lower oxids of nitrogen, and subjecting the said solution thus treat-

20 ed to the action of steam.

9. The process of recovering copper from its ores by the wet method, which comprises 25 leaching the ore with a suitable solvent, treating the resulting solution with a sub- stance containing the lower oxids of nitro-

gen, and subjecting the solution thus treated to the action of a hot fluid blast agent.

10. A step in the process of recovering copper from its ores, which consists in impregnating the copper solution with a substance containing the lower oxids of nitrogen gas. 30

11. A step in the process of recovering copper from its ores, which consists in treating the copper solution with peroxid 35 of nitrogen and the lower oxids of nitrogen.

12. A step in the process of recovering copper from its ores, which consists in treating the copper solution with a substance containing a mixture of peroxid of 40 nitrogen and a lower oxid of nitrogen gas.

In testimony whereof, we have signed our names to this specification, in presence of two subscribing witnesses.

EDWARD SCHAAF.  
STEPHEN G. MARTIN.

Witnesses:

E. E. LONGAN,  
E. L. WALLACE.

Copies of this patent may be obtained for five cents each, by addressing the "Commissioner of Patents,  
Washington, D. C."